

## [54] COLOR COPYING AND SHEET MATERIAL THEREFOR

[75] Inventors: Joseph A. Wiese, Jr.; George Van Dyke Tiers, both of St. Paul, Minn.

[73] Assignee: Minnesota Mining and Manufacturing Company, St. Paul, Minn.

[22] Filed: Feb. 2, 1971

[21] Appl. No.: 111,981

[52] U.S. Cl..... 96/11, 96/67, 96/114.1,  
250/65.1

[51] Int. Cl..... G03c 7/16

[58] Field of Search..... 117/36.8; 96/11,  
96/67, 114.1; 250/65.1

## [56] References Cited

## UNITED STATES PATENTS

2,396,726 3/1946 Trimble ..... 96/11

|           |         |              |          |
|-----------|---------|--------------|----------|
| 3,280,735 | 10/1966 | Clark.....   | 250/65 T |
| 3,301,697 | 1/1967  | Russell..... | 250/65 T |
| 3,370,170 | 2/1968  | Gold.....    | 350/65 T |
| 3,392,020 | 7/1968  | Yutzy.....   | 250/65 T |
| 3,418,468 | 12/1968 | Marx.....    | 250/65 T |
| 3,457,075 | 7/1969  | Morgan.....  | 96/114.1 |
| 3,502,871 | 3/1970  | Marx.....    | 117/36.8 |
| 3,520,691 | 7/1970  | Scheler..... | 117/36.8 |
| 3,531,286 | 9/1970  | Renfrew..... | 117/36.8 |

Primary Examiner—Norman G. Torchin  
 Assistant Examiner—Richard L. Schilling  
 Attorney—Alexander, Sell, Steldt & Delahunt

## [57] ABSTRACT

A stabilized photosensitive heat-developable sheet material or assembly of sheet materials for making color prints or transparencies by a method involving exposure, heat development, and thermographic transfer.

7 Claims, 1 Drawing Figure



PATENTED OCT 23 1973

3,767,394



INVENTORS  
JOSEPH A. WIESE, JR.  
GEORGE VANDYKE TIERS  
BY Kinney, Alexander,  
Sell, Steldt & De Lattu  
ATTORNEYS

## COLOR COPYING AND SHEET MATERIAL THEREFOR

This invention relates generally to the recording of light-images on light-sensitive heat-developable dry silver sheet materials. In one aspect the invention relates to modified dry silver sheet materials and to a method of using the same in making colored prints of colored light-images. In a particular aspect the invention relates to dry silver sheet materials in tri-pack form and to their application in making multi-color prints by a method involving but a single exposure, e.g. through a color negative.

Dry silver sheet materials have been described, in U.S. Pat. No. 3,457,075, as consisting essentially of (a) photosensitive silver halide catalyst-forming means and (b) heat-sensitive reactant image-forming means including an organic silver salt oxidizing agent and a reducing agent for silver ion, the oxidation-reduction reaction of which to produce a visible change is accelerated by said catalyst.

The thermographically induced transfer of volatilizable dyes has been described, e.g., in U.S. Pat. No. 3,280,735, in terms of briefly exposing to intense infrared radiation a printed original, whereby to produce a corresponding heat pattern for volatilizing the dye from a source sheet onto a receptor sheet. The heat pattern is subject to lateral diffusion. The combination of intense light and high temperature has been found in many cases to cause image blurring of imaged dry silver sheet materials under thermographic copying conditions.

It has now been found possible to provide a modified dry silver sheet or coating with which thermographically stable imaged sheets may be produced. It has also been found possible to employ such sheet materials in a thermographic image transfer process whereby to produce sharply defined monicolor or multicolor prints of colored light images, all as will hereinafter be set forth.

The single FIGURE of the drawing represents in cross-section a portion of a pack of modified dry silver sheets prepared in accordance with the principles of the invention and useful in making full-color prints.

Sheet 10 comprises a transparent film support 11 having on one surface a modified dry silver coating 12 and on the other surface a volatilizable dye 13. Similarly, sheet 14 comprises film 15, dry silver coating 16 and dye coat 17, and sheet 18 comprises film 19, dry silver coating 20 and dye coating 21. The three sheets, assembled as shown, comprise a tripack 22.

In making a print, the tripack 22 is first exposed to a light-image from the upper surface as seen in the drawing. After exposure the three sheets are heated briefly to develop in each a dense image corresponding to a portion of the light-image, and the three are then successively placed in registry against a receptor sheet and the composite is briefly exposed to intense infrared radiation, e.g., in a thermographic copying machine. The heat patterns induced in the image areas cause transfer of dye to corresponding areas of the receptor sheet, with production of a colored image. Alternatively, the separate dye images are transferred to separate transparent film receptor sheets which are then placed in registry to form a full-color transparency.

In a modification of the method just described, and using a dry silver composition which under appropriate

development conditions has a negative D log E slope, the exposed sheets are developed in a manner to produce a positive rather than a negative image. The resulting dye images obtained by thermographic transfer from the thus imaged films then represent a direct rather than a color reversed record of the initial colored light pattern.

The dry silver coatings 12, 16 and 20 are respectively sensitized to blue, green and red light, as indicated in the drawing by the letters B, G and R. The dye coatings 13, 17 and 21 analogously contain yellow, magenta and cyan dyes respectively, indicated as Y, M and C. The transparent carrier film is marked T in each instance. The dye layers assist in absorbing light other than that to which the lower layer or layers of dry silver material have been sensitized, so that a sharp separation of color is accomplished and a true showing of both white and black as well as color is accomplished in the final print or print assembly. The lower dye layers also serve as antihalation layers and assist in providing sharply defined images.

As above indicated, both direct and reverse light patterns may be reproduced as direct color prints. Thus the light pattern may be obtained either by direct reflection from a colored subject or colored original, or by projection through a colored transparency which may be either a positive or a negative photographic color transparency.

An important feature of the invention resides in the stabilizing of the imaged dry silver layer against further darkening of the background, or lateral spreading of the image areas, under continued heating or exposure to infra-red. It has been found that various halogen-containing organic oxidizing agents may be incorporated in the dry silver coatings without altering the initial light-sensitivity thereof, and that such compounds effectively stabilize the imaged sheet.

Compounds in which a positive halogen is attached directly to nitrogen represent a particularly effective class of stabilizers. Compounds such as N-bromosuccinimide and N,N'-dichloro-N,N'-dibenzoylethylenediamine are representative. This compound also known as N,N'-dichloro-1,2-ethylene bisbenzamide, is a presently preferred stabilizer material. The stabilizer may be incorporated in a composition containing all of the required components for preparing the photosensitive heat-developable dry silver coating. The more active stabilizers are preferably added in a second coating, the photosensitive components being applied in a separate first coating, to avoid any tendency toward desensitization of the photosensitive materials prior to heat development.

The following specific Example will serve as a further illustration of the principles of the invention.

### EXAMPLE

A first composition is prepared by first dispersing 20 parts by weight of silver behenate full soap in a mixture of 37.5 parts methylcelulose ketone and 42.5 parts toluene, preferably by prolonged ball milling. To 50 gms. of the dispersion is added 40 ml. of methyl isobutyl ketone, 10 ml. of a 2% solution of mercuric bromide in methyl alcohol, and 22 gms. of a 15% solution of polyvinylbutyral resin in ethyl alcohol, all operations beginning with addition of mercuric bromide being conducted under darkroom conditions. To such mixtures are then added various spectral sensitizer materi-

als, and each of the resulting mixtures is coated on two mil Mylar polyester film at a wet thickness of three mils, and permitted to dry.

Three separate sensitizers are used the composition and amounts of which are as follows:

Blue Sensitizer: add 4.5 ml. of a .05% solution in acetone.



Green Sensitizer: add 3 ml. of a .05% solution in acetone.



Red Sensitizer: add 6 ml. of a .05% solution in methanol.



Over the above coatings is then supplied a further coating consisting of the following:

3% solution of cellulose acetate butyrate in methyl-ethyl ketone—75 ml.

20% solution of polymethylmethacrylate in ethyl acetate—10 ml.

phthalazinone—1 gm.

2,2'-methylenebis-(4-methyl-6-tertiary-butyphenol)—4 gm.

2% solution of phthalic acid in methanol—1.5 ml.

N,N'-dichloro-1,2-ethylene bisbenzamide—2.75 gm.

The second coating is likewise applied at a wet thickness of 3 mils and dried.

The reverse surfaces of the three coated films are then separately coated with the appropriate dyes, the coating solutions in each instance consisting of 326 mgm. of dye in 10 gms. of a 16.7% solution of acrylonitrile:vinylidene copolymer (Saran F-220) in methyl-ethyl ketone. The yellow dye is Sudan Yellow GR Concentrate, Color Index 21240. The magenta dye is 4-tricyanovinyl-N,N-di-n-butylaniline. The cyan dye is DuPont Oil Blue A, Color Index Solvent Blue 36. Other useful volatilizable dyes include Sudan Yellow RRA, Sudan Yellow GGA, Special Red S Conc., and Smoke Green No. 1.

The three coated films are combined in a tri-pack in the relationship shown in the drawing, and the pack is

exposed to a reverse color light-image by contact printing through a photographic color negative. The three films are separately briefly heated to form on each a dense visible image at the light-struck areas. The films

5 are then laid against transparent polymeric receptor films, in this case consisting of thin transparent Mylar polyester film lightly coated with a mixture of 1.5 grams of nickel acetate tetrahydrate and 10 grams of polyvinyl alcohol applied from solution in 90 grams of 10 water, and are briefly exposed to intense infra-red radiation in a thermographic copying machine to form on each receptor a monicolor partial negative image. The three imaged receptor films are placed together in registry to provide a full color positive transparency.

15 Another tripack assembly is first exposed to a direct color light-image by contact printing through a photographic color positive serving as an original, and the three films are separately subjected to minimum heat required to produce maximum useful density at unex-

20 posed areas. By such continued heating the initially darkened light-struck areas are transparentized while the initially transparent non-light-struck areas progressively darken to a maximum. The three films are then successively placed against a receptor sheet consisting

25 of white paper lightly coated with a mixture of four parts by weight of calcium stearate, two parts of nickel stearate, four parts of calcium carbonate, and ten parts of polyvinyl alcohol, applied in 90 parts of water. The composite is in each case passed through the thermo-

30 graphic copying machine, the imaged film in each case being placed in registry with the position of any preceding imaged film or films. A direct full-color reproduction of the colored original is obtained.

In the foregoing Example, exposure is typically between 3 and 6 seconds using as the light source a 650 watt FAB tungsten filament quartz iodine lamp at a distance of 3 feet, and development is achieved by heating at temperatures between about 125° and 135° C. With other formulations and conditions it may be found necessary to modify these values, but the necessary modifications are readily determined by simple preliminary sensitometric test procedures well within the skill of the art.

What is claimed is as follows:

45 1. A photosensitive sheet material comprising a transparent thin carrier having over one surface a photosensitive heat developable dry silver layer comprising (a) photosensitive silver halide catalyst-forming means, (b) heat-sensitive reactant image-forming means including an organic silver salt oxidizing agent and a reducing agent for silver ion, the oxidation-reduction reaction of which to produce a visible change is accelerated by said catalyst, and (c) N,N'-dichloro-1,2-ethylenbisbenzamide or N-bromosuccinimide, and said carrier having over the other surface a layer comprising, in a polymeric binder, a dye which is volatilizable therefrom at temperatures obtained under thermographic copying conditions.

55 2. Sheet material of claim 1 wherein said dry silver layer contains a spectral sensitizer for sensitizing said sheet to a primary color.

60 3. A pack of sheet material useful in making full-color prints and comprised of three sheets of photosensitive sheet material each comprising a transparent thin carrier having over one surface a heat-stabilized photosensitive heat developable dry silver layer comprising (a) photosensitive silver halide catalyst-forming means

and (b) heat-sensitive reactant image-forming means including an organic silver salt oxidizing agent and a reducing agent for silver ion, the oxidation-reduction reaction of which to produce a visible change is accelerated by said catalyst, and (c) a spectral sensitizer for sensitizing said sheet to a primary color, and said carrier having over the other surface a layer comprising, in a polymeric binder, a dye which is volatilizable therefrom at temperatures obtainable under thermographic copying conditions, and wherein the first of said three sheets carries a cyan dye and is sensitized to red, the second carries a magenta dye and is sensitized to green, and the third carries a yellow dye and is sensitized to blue.

4. A pack of sheets according to claim 3 wherein the dry silver layers each contain N,N'-dichloro-1,2-ethylene-bisbenzamide or N-bromosuccinimide.

5. Method of making a multicolor print comprising: (1) exposing to a light-image a pack of three sheets of photosensitive sheet material each comprising a transparent thin carrier having over one surface a heat-stabilized photosensitive heat developable dry silver layer comprising (a) photosensitive silver halide catalyst-forming means and (b) heat-sensitive reactant image-forming means including an organic silver salt oxidizing agent and a reducing agent for silver ion, the oxidation-reduction reaction of which to produce a visible change is accelerated by said catalyst, and (c) a spectral sensitizer for sensitizing said sheet to a primary color, and said carrier having over the other surface a layer comprising, in a polymeric binder, a dye which is volatilizable therefrom at temperatures obtainable under thermographic copying conditions, and wherein the first of said three sheets carries a cyan dye and is

sensitized to red, the second carries a magenta dye and is sensitized to green, and the third carries a yellow dye and is sensitized to blue, with said light-image being incident on said third sheet; (2) separating the three sheets and heating each one independently to develop a visible image; and (3) separately briefly exposing each sheet to intense infra-red radiation while maintaining the dye layer against a common receptor sheet and with each sheet in registry with the position of the preceding sheet or sheets.

6. Method of claim 5 wherein the receptor sheet includes a surface coating comprising a nickel salt of an organic acid in a water-soluble binder.

7. Method of making a color print comprising: exposing to a light-image a photosensitive sheet material comprising a transparent thin carrier having over one surface a photosensitive heat developable dry silver layer comprising (a) photosensitive silver halide catalyst-forming means, (b) heat-sensitive reactant image-forming means including an organic silver salt oxidizing agent and a reducing agent for silver ion, the oxidation-reduction reaction of which to produce a visible change is accelerated by said catalyst, and (c) N,N'-dichloro-1,2-ethylenebisbenzamide or N-bromosuccinimide, and said carrier having over the other surface a layer comprising, in a polymeric binder, a dye which is volatilizable therefrom at temperatures obtained under thermographic copying conditions; heating the exposed sheet to develop a visible image; and briefly exposing the imaged surface to intense infrared radiation while maintaining the dye-carrying surface against a receptor sheet.

\* \* \* \* \*

UNITED STATES PATENT OFFICE  
CERTIFICATE OF CORRECTION

Patent No. 3,767,394

Dated Oct. 23, 1973

Inventor(s) Joseph A. Wiese, Jr. and George Van Dyke Tiers

It is certified that error appears in the above-identified patent  
and that said Letters Patent are hereby corrected as shown below:

Column 3, lines 21-30

The structural formula of the green sensitizer  
should be:



Signed and sealed this 9th day of April 1974.

(SEAL)

Attest:

EDWARD M. FLETCHER, JR.

C. MARSHALL DANN  
Commissioner of Patents